

## 1

3,222,281

OXIDATION INHIBITORS FOR LUBRICANT OILS  
 Edwin L. De Young, Milwaukee, Wis., and Roger W. Watson, Highland, Ind., assignors to Standard Oil Company, Chicago, Ill., a corporation of Indiana  
 No Drawing. Filed Jan. 16, 1962, Ser. No. 167,221  
 8 Claims. (Cl. 252—49.6)

This invention relates to novel oxidation inhibitors for hydrocarbon lubricant oils. More particularly, it provides a unique organosilicon compound having a remarkable effectiveness for inhibiting such oxidation.

It has now been discovered, pursuant to the invention, that an outstanding oxidation inhibitor for hydrocarbon lubricant oils comprises the reaction product of an aldehyde having up to about 20 carbon atoms per molecule with silicon disulfide. The reaction product, in addition to its efficacy for the foregoing purpose, is relatively stable, oil soluble, and producible from low-cost reactants and with minimum difficulty.

The starting aldehyde may be any of the relatively low molecular weight aldehydes, that is, having up to about 20 carbon atoms per molecule and having the formula RCHO, with the group R which is attached to the carbonyl group being preferably alkyl, but also alkenyl, substituted alkyl, aryl, aralkyl, or alkaryl. As illustrative non-limiting examples of suitable aldehydes there may be mentioned: formaldehyde (which is not, however, reactable in certain polymeric forms such as paraformaldehyde), acetaldehyde, propionaldehyde, n-butyraldehyde, isobutyraldehyde, n-valeraldehyde, n-caproaldehyde, n-heptaldehyde, acrolein, crotonaldehyde, chloral, chloral hydrate, benzaldehyde, tolualdehyde, etc. The aldehyde reactant is advantageously employed in large excess over the silicon disulfide.

Anhydrous conditions are apparently preferred during the reaction. Water evidently decomposes silicon disulfide to a silicon oxide or hydroxide and hydrogen sulfide, thus making it unavailable for the reaction. A temperature within the range of about 50 to about 150° C., optimally around 100–130° C., is desirably employed, and is maintained for a sufficient time to permit substantial cessation of hydrogen sulfide evolution. Temperatures higher or lower than those cited previously may be employed, although it appears that lower temperatures unduly tend to increase reaction time while there is no particular advantage in operating at higher temperatures.

The inventive oxidation inhibitor may be employed in hydrocarbon lubricant oils in concentrations ranging from as low as 0.05 weight percent to about 3 percent or even higher. The precise concentration depends upon the intrinsic corrosivity of the lubricant oil together with the extent of inhibition desired, and may be determined from sample tests.

Hydrocarbon lubricant oils are generally those naturally or synthetically derived (e.g., propylene polymer or isobutylene polymer oils) having viscosity ranging from about 20 S.S.U. at 100° F. to about 3,000 S.S.U. at 210° F. Such oils may contain various other additives such as detergents, viscosity index improvers, pour points, depressants, extreme pressure additives, foam inhibitors, dyes, etc.

The inventive inhibitors may be evaluated quantitatively by means of the Stirring Sand Corrosion Test (S.S.C.T.).

For the S.S.C.T., a copper-lead test specimen is lightly abraded with steel wool, washed with naphtha, dried and weighed to the nearest milligram. The cleaned copper-lead test specimen is suspended in a steel beaker, cleaned with a hot tri-sodium phosphate solution, rinsed with water, acetone and dried, and 250 grams of the oil to be tested, together with 0.625 gram lead oxide and 50 grams

## 2

of a 30–35 mesh sand charged to the beaker. The beaker is then placed in a bath or heating block and heated to a temperature of 300° F. (plus or minus 2° F.) while the contents are stirred by means of a stirrer rotating at 750 r.p.m. The contents of the beaker are maintained at this temperature for 24 hours, after which the copper-lead test specimen is removed, rinsed with naphtha, dried and weighed. The test specimen is then replaced in the beaker and an additional 0.375 gram of lead oxide added to the test oil. At the end of an additional 24 hours of test operation the test specimen is again removed, rinsed and dried as before, and weighed. The test specimen is again placed in the beaker together with an additional 0.250 gram of lead oxide and the test continued for another 24 hours (72 hours total). At the conclusion of this time, the test specimen is removed from the beaker, rinsed in naphtha, dried and weighed. The loss in weight of the test specimen is recorded after each weighing. A weight loss of 200 milligrams or less in 48 hours and 500 milligrams or less in 72 hours is allowable.

The invention may be illustrated with reference to the following embodiments, which are intended to illustrate the principles of the invention but not to be wholly exclusive or definitive with respect to scope or conditions.

## Example 1

This example illustrates the preparation of the reaction product of silicon disulfide and n-heptaldehyde.

To a flask containing 22.8 grams (0.2 mol) of technical n-heptaldehyde is added 9.2 grams (0.1 mol) of finely powdered silicon disulfide. The mixture is stirred at 100–110° C. for 5 hours until hydrogen sulfide is no longer evolved. The hot mixture is filtered and the filtrate evaporated under vacuum to remove unreacted n-heptaldehyde. The product is a gelatinous solid containing 5.0 weight percent silicon.

When added to a heavy-duty S.A.E. 30 base oil at a concentration of only 0.5 weight percent, the additive produced above exhibits a weight loss of only 90.3 milligrams at 48 hours and 88.4 milligrams at 72 hours.

The additive prepared in this example, when contrasted with a somewhat similar additive prepared by reacting silicon sulfide with methyl-n-heptyl ketone is demonstrated by comparing the two products with respect to their performance under the S.S.C.T. and under the silver ball Falex test (Journ. Inst. Pet., 32, April 1946); the present additive is almost three times as effective as the ketone-prepared additive under the conditions of the S.S.C.T., while it is only about a fifth as effective in reducing silver wear in the silver Falex test.

## Example 2

Example 1 is repeated with acetaldehyde, in an equal molar quantity, substituting for the n-heptaldehyde. The reaction is conducted under pressure to maintain a liquid phase. Excellent results are obtained under the S.S.C.T.

## Example 3

Example 1 is repeated with isobutyraldehyde, a mixture of n-heptaldehyde with formaldehyde, acrolein, chloral, benzaldehyde, and p-chloro-benzaldehyde. The resultant products are all effective oxidation inhibitors under the conditions of the S.S.C.T.

Thus it is apparent from the foregoing description that there has been provided an outstanding oxidation inhibitor for hydrocarbon lubricant oils. While the invention has been described in conjunction with certain embodiments thereof, it is manifest that these are by way of illustration only, and that various alternatives, modifications, and variations will become apparent to those skilled in the art in light of the foregoing description. Accordingly, it is intended to embrace all such alternatives, modifica-

tions, and variations as fall within the spirit and broad scope of the appended claims.

We claim:

1. A hydrocarbon lubricating oil normally susceptible to oxidation containing, in a minor amount sufficient to inhibit said oxidation, the reaction product obtained by reacting a C<sub>1-20</sub> aldehyde and silicon disulfide in a molar ratio of from about 1-2 moles of said aldehyde per mole of said disulfide under anhydrous conditions at a temperature of from about 50 to about 150° C. until hydrogen sulfide is no longer evolved, said aldehyde having the formula RCHO wherein R is a member of the group consisting of alkyl, chloro-substituted alkyl, alkenyl, phenyl, chlorophenyl and tolyl.

2. The lubricant of claim 1 wherein the amount of said reaction product is from about 0.05 to about 3 weight percent.

3. The lubricant of claim 2 wherein R is C<sub>1-12</sub> alkyl.

4. The lubricant of claim 2 wherein said aldehyde is n-heptaldehyde.

5. The reaction product obtained by reacting a C<sub>1-20</sub> aldehyde and silicon disulfide in a molar ratio of from about 1-2 moles of said aldehyde per mole of said disulfide under anhydrous conditions at a temperature of from about 50 to about 150° C. until hydrogen sulfide is no longer evolved, said aldehyde having the formula

RCHO wherein R is a member of the group consisting of alkyl, chloro-substituted alkyl, alkenyl, phenyl, chlorophenyl and tolyl.

6. The composition of claim 5 wherein R is C<sub>1-12</sub> alkyl.

7. The composition of claim 5 wherein said aldehyde is n-heptaldehyde.

8. The method of preparing a composition suitable for use as an oxidation inhibitor for hydrocarbon lubricating oils which comprises reacting C<sub>1-20</sub> aldehyde and silicon disulfide in a molar ratio of from about 1-2 moles of said aldehyde per mole of said disulfide under anhydrous conditions at a temperature of from about 50 to about 150° C. until hydrogen sulfide is no longer evolved, said aldehyde having the formula RCHO wherein R is a member of the group consisting of alkyl, chloro-substituted alkyl, alkenyl, phenyl, chlorophenyl and tolyl; and recovering the resultant composition.

20

References Cited by the Examiner

UNITED STATES PATENTS

2,588,083 3/1952 Burkhard et al. \_\_\_\_ 260—448.2

25 DANIEL E. WYMAN, Primary Examiner.

ALPHONSO D. SULLIVAN, Examiner.